

March 9, 1954

D. B. WESTCOTT ET AL

2,671,727

## MANUFACTURE OF PULP BY THE ALKALINE PROCESS

Filed May 5, 1948



INVENTORS  
DANA B. WESTCOTT  
HAROLD FIELD  
BY  
Moses, Nolte, Creasey & Perry  
ATTORNEYS

## UNITED STATES PATENT OFFICE

2,671,727

MANUFACTURE OF PULP BY THE  
ALKALINE PROCESS

Dana B. Westcott and Harold L. Field, Mechanicville, N. Y., assignors to West Virginia Pulp and Paper Company, New York, N. Y., a corporation of Delaware

Application May 5, 1948, Serial No. 25,226

8 Claims. (Cl. 92—9)

1

Our present invention relates to the manufacture of pulp from wood and other suitable fibrous materials.

In general, it is the object of our invention to devise an improved process of cooking in which the raw cellulosic material will be subject to conditions of great uniformity whereby a pulp of high uniform quality will be produced. It is a further object to provide a process of cooking which will be more economical to operate.

In carrying out our improved process we preferably provide for the operation of a multiple of digesters served by a single accumulator for cooking liquor through which and through each digester in operation a continuous circulation of liquor is had. We further constantly maintain the active alkali concentration and temperature of the liquor entering the digesters at predetermined, preferably low optimum values preferably by continuously fortifying the liquor prior to its admission to the digesters both with active alkali and with heat. Furthermore by passing the liquor through the digesters in parallel sufficiently rapidly, the drop in active alkali concentration and that in heat content will be kept within narrow predetermined limits. When the cooking of a charge in a given digester is complete such digester is cut out of the system and blown.

Cooking a charge by bathing it in a flowing stream of cooking liquor which is continuously maintained within an optimum range of active alkali and of temperature has signal advantages, among which may be mentioned (1) a higher grade of pulp as indicated by a higher viscosity number due to the absence of high initial alkali concentrations as is the practice in the ordinary cooking operation and also to the fact that there is less pulp which is either overcooked or undercooked; (2) greater use of the digester capacity inasmuch as the digester may be completely packed full of chips; (3) since the cooking liquor is continuously fortified it is possible to use the liquor until it has a greater solids content before sending it to the evaporators with substantial economies in evaporator operation; (4) the system results in cleaner blows; (5) complete submergence of the chips is had since the digester is fully charged with liquor; (6) there is no need to weigh or measure the amount of chips charged the digester or to determine in advance the moisture content of the charge.

While multiple operation of digesters has heretofore been proposed, such multiple operation has not been had so far as we are aware, in which the active alkali concentration of the cooking

2

liquor is continuously maintained within optimum limits. Furthermore while the so-called injection cooking, i. e., injecting concentrated alkali into the circulating liquor from time to time has been proposed the advantages of quick heating of the chips by charging with already heated liquor available in multiple digester operation as well as other of the above advantages have not been realized.

10 Our invention will be best understood by reference to the following detailed description of an illustrative example taken with the annexed drawing, the single figure of which shows a hook-up of several digesters and an accumulator 15 adapted for carrying out the improved process.

In the drawing, there are shown digesters 1, 2, 3, 4 and 5, each of which is in communication with an accumulator 6 by means of pipe 7 connected to the top of each digester by valved branch pipes 1a respectively; the return flow from the accumulator passes through pipe 8 and thence into offtakes 1a, 1b, 1c, 1d, 1e, respectively leading to the bottom of digesters 1 to 5. Each of said offtakes has in its circuit a pump 9 and 20 a heater 10. Each of said heaters is of the heat exchanger type in which the charge is indirectly heated by steam admitted thereto by connections not shown. Each digester has a strainer 8a preferably located in the extreme top thereof.

25 Fresh white liquor for maintaining the active chemical concentration is admitted, preferably continuously, to the volume of liquor in circulation by means of pipe 11 which joins pipe 8. Spent black liquor from the pulp washers (not shown) is similarly admitted through pipe 11a and serves to maintain the necessary volumetric level. The feed rates of both the white liquor and black liquor injected can, if desired, be made 30 fully automatic. Since the active soda concentration is a direct function of the electrical conductivity of the cooking liquor, the active soda concentration may be maintained at a fixed level automatically by a conductivity controller 12 of known construction which measures the conductivity of a small sample of cooking liquor withdrawn continuously from pipe 8 through pipe 12a at a point after the new chemicals are added, and 35 controls this measured conductivity at a fixed point by actuating motorized valve 12b placed on pipe 11. A mixing chamber 12c may also be provided in line 8 and may contain a 40 motorized stirrer not shown whereby to insure thorough mixing of the added liquors. A differential pressure type level controller 13 suitably connected to accumulator 6 by piping 13a may

45 50

be used to measure the level in the accumulator and control this level between a suitable range by energizing a motorized valve 13b on the black liquor pipe 11a.

The air charged with the chips and any gases produced during the pulping reaction are carried by the circulating liquor from the digesters 1-5 to the accumulator 6. These gases are continuously relieved to the atmosphere from one point, line 14. A suitable bypass line 15 is had whereby the accumulator charge may be heated in heater 10 when first starting up the system. In the hook-up shown each digester had a capacity of 808 cu. ft. and when completely filled held from 6,000 to 10,000 pounds (depending upon its density) of chipped wood on an oven dried basis, such wood consisting of coniferous or deciduous species or mixtures of the two and containing 30 to 55% moisture.

In the example, the description of which now follows, approximately 10,000 pounds (O. D. basis) of mixed hardwood chips containing 35% moisture were charged to the digester (1) and the cover bolted on. 6000 gallons (at 20° C.) of spent black liquor at the temperature available was charged to the accumulator 6 through pipe 11a. The composition of this liquor was as follows:

|                                                    | Grams per liter |
|----------------------------------------------------|-----------------|
| Active soda as Na <sub>2</sub> O                   | 7.7             |
| Total soda as Na <sub>2</sub> O                    | 52.0            |
| Organic matter                                     | 125.7           |
| Total solids                                       | 192.8           |
| Sulfidity (Na <sub>2</sub> S as Na <sub>2</sub> O) | 3.0             |

The liquor charge in the accumulator 6 was heated to 150° C. by pumping out of the bottom of the accumulator through pipe 8 and pipe 1a, through heater 10 and through bypass pipe 15 back to the top of the accumulator. While this liquor was being heated, an amount of white liquor at 120 g./l. active Na<sub>2</sub>O concentration was added to pipe 8 through pipe 11 to raise the cooking liquor to 10 g./l. active Na<sub>2</sub>O as measured by the conductivity meter. This required about 125 gallons of white liquor to effect this increase in concentration of active soda. When the liquor in the accumulator had reached 150° C. temperature and 10 g./l. active soda, the digester 1 was charged with this liquor by opening the valves at the bottom and top of the digester and closing the valve in the bypass line 15. The pump 9 on digester 1 forced this liquor through the digester and back to the accumulator at a rate of approximately 500 gallons per minute. When the digester was full of liquor and the liquor was flowing back to the accumulator, 5200 gallons of the original accumulator liquor charge was in the digester 1 and about 925 gallons in the accumulator 6.

Also, as soon as liquor from digester 1 began to return to the accumulator 6 and then started to flow back to the digester 1, the active soda concentration fell off to about 4 g./l. or above due to dilution of the liquor with wood moisture and to reaction of the active chemical with the wood. The active soda concentration was then built up to its original 10 g./l. by injection of white liquor through pipe 11. In this manner, the liquor entering the bottom of digester 1 was maintained at 10 g./l. active Na<sub>2</sub>O concentration throughout the six hour cook after which the digester was blown. Naturally the amount of white liquor added to maintain the Na<sub>2</sub>O concentration of the entering liquor diminished as the cook proceeded.

In like manner, the temperature of the liquor entering the digester 1 was maintained at a constant value of 150° C. From 45 to 60 minutes were required to bring the contents up to 150° C.

Therefore, during at least five hours of the entire six hour cooking period the wood in the digester was subjected to a cooking liquor maintained at substantially the same temperature and active chemical concentration.

10 A total of 2000 gallons of white liquor of 120 g./l. active Na<sub>2</sub>O was required for this six hour cook; 125 gallons to raise the accumulator charge to 10 g./l. and 1875 gallons for injection during the cook to maintain the concentration at

15 10 g./l. During the cook 2680 gallons of black liquor were added at a uniform rate through pipe 11a. A total of 4555 gallons of hot white and black liquor were then added in order to have the accumulator at full charge by the end of the cook and ready to charge another cook in another digester of the battery. Similarly the accumulator will be charged sufficiently to fill any digester whenever it is ready to be cut into the system.

20 During the 6-hour cook, 180,000 gallons of liquor were circulated. Approximately .52 gallon of liquor at room temperature is required to cover a pound of hard wood chips on an O. D. basis. Hence the minimum amount of liquor necessary to start with is 5200 gallons for 10,000 pounds of hard wood chips. Dividing the total number of gallons pumped, 180,000 by the number of gallons necessary to cover the chips it will be seen that approximately 35 times the volume of liquor necessary to cover the chips is circulated during the cook.

The pulp so produced from mixed hard woods had the following properties:

25 40 Permanganate number ----- 13.8  
Viscosity<sup>1</sup> ----- cp 5,550  
Screenings on basis of screened pulp obtained, less than 5.4%

30 45 Tappi: A 1.25% solution of the pulp in 0.5 molar cupriethylene diamine is first formed and its viscosity then measured by the falling ball method.

A total of 0.2 pound (91 grams) of active soda per pound of O. D. wood was applied during the cook, this soda being added as a kraft white liquor containing 116 g./l. NaOH and 38 g./l. Na<sub>2</sub>S. As is customary both the sodium hydroxide and the sodium sulfide are expressed in terms of Na<sub>2</sub>O and the total of the two constitute the active Na<sub>2</sub>O concentration in the cooking liquor.

55 55 The high viscosity of the unbleached pulp was evidence that the cellulose had undergone relatively little degradation and that the pulp would have a high strength (we have found that if the viscosity of the unbleached pulp falls below 2000 centipoises, the strength is inferior. Otherwise

60 expressed, the fall of strength with fall of viscosity proceeds at an accelerated rate below 2000 cp.). In the present process the high viscosity obtained is attributable to the low active

65 Na<sub>2</sub>O concentration of the cooking liquor, to the comparatively low temperature of the cook and the uniformity of the cooking conditions. If desired the temperature of the cook may be raised from a minimum, say of 145° C. to 175° as the upper limit, with a shortening of the time of cook, but the pulp will have a decreased viscosity. Similarly the quality of the pulp will undergo a change when the concentration of the active alkali is increased. Whatever change is

70 75 brought about by variation of temperature and

concentration of chemicals the pulp produced is of uniform quality. For best results we have found that the active alkali concentration of the cooking liquor as it enters the digester should be not substantially less than 10 g./l. and not substantially more than 20 g./l.

It will be noted that although the quantities are here given for the sake of completeness, it is not necessary to weigh the chips added to the digester nor is it necessary to know their moisture content, since the liquor entering the digester will be maintained at the same concentration of active chemicals.

When operating the battery of five digesters shown, after No. 1 digester has been started, digester No. 2, after having been filled with chips is started up after a suitable interval, say 81 minutes from the time that digester No. 1 was started by pumping thereto liquor through the pipe 1b. The black liquor injection rate must be increased enough so that the accumulator is full and ready to charge in 81 minutes, using a 6-hour length of cook. Also sufficient white liquor will be added to the accumulator through pipe 1b to maintain the concentration at 10 g./l. Na<sub>2</sub>O or other predetermined value. Similarly, each of the other digesters 3, 4 and 5 will be filled with chips and cut into the system each one following the other after the same time interval.

When a newly filled digester is cut into the system the liquor which is first passed therethrough is naturally cooled considerably and diluted by the moisture in the chips. However, this dilution and loss of heat will be easily made up by reason of the fact that the diluted liquor is mingled with the liquor in circulation from the other digesters which in effect function as accumulators. Likewise the steam demand of the system is made much more uniform than if a single digester were being employed.

If desired the process may be carried out with the combination of an accumulator and a single digester with, however, corresponding loss of operating efficiency.

We claim:

1. The method of cooking wood to obtain pulp therefrom, which comprises the steps of filling a plurality of digesters with wood chips, maintaining a continuous flowing stream of alkali cooking liquor through said digesters in parallel and through an accumulator, the wood in each digester being maintained submerged in a flowing body of liquor, the liquor having a temperature in the range of about 145° C. to about 175° C. and having an effective Na<sub>2</sub>O content in the range of from about ten grams per liter to about twenty grams per liter, substantially continuously assaying the stream of liquor leaving the accumulator on its way to said plurality of digesters for effective alkali content and temperature, restoring depleted Na<sub>2</sub>O and heat values to said liquor in response to said assay to maintain the same within the said ranges, blowing each of said digesters sequentially after completion of the cook therein while maintaining the stream through the remaining digesters and accumulator, filling each blown digester with wood chips and connecting the same to the stream, subjecting the wood in the last named digester to the action of the stream at the said cooking temperature and alkali content thereby quickly bringing the same to cooking temperature, and accomplishing the cooking thereof as above set forth.

2. The method of cooking wood to obtain pulp therefrom, which comprises the steps of filling

a plurality of digesters with wood chips, maintaining a continuous flowing stream of alkali cooking liquor through said digesters in parallel and through an accumulator, the wood in each digester being maintained submerged in a flowing body of liquor, the liquor having a temperature in the range of about 145° C. to about 175° C., the said stream having an effective Na<sub>2</sub>O content in the range of from about ten grams per liter to about twenty grams per liter when entering the digester, the rate of flow of said stream being such that said Na<sub>2</sub>O content is maintained at not less than four grams per liter at the outlet end of the digesters, substantially continuously assaying the stream of liquor leaving the accumulator on its way to said plurality of digesters for effective alkali content and temperature, restoring depleted Na<sub>2</sub>O and heat values to said liquor in response to said assay, blowing each of said digesters sequentially after completion of the cook therein while maintaining the stream through the remaining digesters and accumulator, filling each blown digester with wood chips and connecting the same to the stream, subjecting the wood in the last named digester to the action of the stream at the said cooking temperature thereby quickly bringing the same to cooking temperature, and accomplishing the cooking thereof as above set forth.

3. The method of cooking wood to obtain pulp therefrom, which comprises the steps of filling a plurality of digesters with wood chips, maintaining a continuous flowing stream of alkali cooking liquor through said digesters in parallel and through an accumulator, the wood in each digester being maintained submerged in a flowing body of liquor, the liquor having a temperature in the range of about 145° C. to about 175° C. and having an effective Na<sub>2</sub>O content in the range of from about ten grams per liter to about twenty grams per liter, restoring depleted alkali and heat to said stream of liquor leaving the accumulator on its way to said plurality of digesters, blowing each of said digesters sequentially after completion of the cook therein while maintaining the stream through the remaining digesters and accumulator, filling each blown digester with wood chips and connecting the same to the stream, subjecting the wood in the last named digester to the action of the stream at the said cooking temperature and alkali content thereby quickly bringing the same to cooking temperature, and accomplishing the cooking thereof as above set forth.

4. The method of cooking wood to obtain pulp therefrom, which comprises the steps of filling a plurality of digesters with wood chips, maintaining a continuous flowing stream of alkali cooking liquor through said digesters in parallel and through an accumulator, the wood in each digester being maintained submerged in a flowing body of liquor, the liquor having a temperature in the range of about 145° C. to about 175° C., the said stream having an effective Na<sub>2</sub>O content in the range of from about ten grams per liter to about twenty grams per liter when entering the digester, the rate of flow of said stream being such that said Na<sub>2</sub>O content is maintained at not less than four grams per liter at the outlet end of the digesters, restoring depleted heat values and alkali content to the stream of liquor leaving the accumulator on its way to said plurality of digesters, blowing each of said digesters sequentially after completion of the cook therein while maintaining the stream through the re-

maining digesters and accumulator, filling each blown digester with wood chips and connecting the same to the stream, subjecting the wood in the last named digester to the action of said stream at the said cooking temperature thereby quickly bringing the same to cooking temperature, and accomplishing the cooking thereof as above set forth.

5. The method of claim 3 in which the cooking liquor is a kraft liquor.

6. The method of claim 3 in which the flow of the liquor is upwardly through said digesters.

7. The method of claim 4 in which the cooking liquor is a kraft liquor.

8. The method of claim 4 in which the flow of 15 the liquor is upwardly through the digesters.

DANA B. WESTCOTT.  
HAROLD L. FIELD.

## References Cited in the file of this patent

## UNITED STATES PATENTS

| Number    | Name           | Date          |
|-----------|----------------|---------------|
| 882,790   | Muntzing       | Mar. 24, 1908 |
| 1,690,954 | Spencer        | Nov. 6, 1928  |
| 1,784,849 | Richter        | Dec. 16, 1930 |
| 1,887,899 | Bradley et al. | Nov. 15, 1932 |
| 1,918,459 | Dunbar et al.  | July 18, 1933 |
| 2,190,193 | Richter        | Feb. 13, 1940 |

## FOREIGN PATENTS

| Number  | Country | Date         |
|---------|---------|--------------|
| 441,890 | Canada  | June 3, 1947 |

## OTHER REFERENCES

Wells et al. article in Paper Trade Journal, pp. 30-36, November 9, 1944.

Wells article in Paper Trade Journal, pp. 42-46, October 30, 1947.